

June 6, 1944.

J. E. JOHNSON

**2,350,899**

## PROCESS OF PRODUCING CASTINGS

Original Filed April 18, 1940 2 Sheets-Sheet 1



*Inventor:*  
JOSEPH E. JOHNSON  
*Attorneys*  
TOWNSEND & DECKER.

June 6, 1944.

J. E. JOHNSON

2,350,899

PROCESS OF PRODUCING CASTINGS

Original Filed April 18, 1940 2 Sheets-Sheet 2



Inventor:  
JOSEPH E. JOHNSON

By *Townsend & Walker*  
Attorneys

## UNITED STATES PATENT OFFICE

2,350,899

## PROCESS OF PRODUCING CASTINGS

Joseph E. Johnson, Brooklyn, N. Y.

Original application April 18, 1940, Serial No. 330,287. Divided and this application December 28, 1942, Serial No. 470,354

10 Claims. (Cl. 22—200)

This invention has for its principal object the production, by an expeditious, facile and novel method or process, of an exact and faithful reproduction or facsimile of an object, such as an insignia, inscription, cameo, intaglio etc. which has been placed in a die or which forms a part thereof. The invention is peculiarly adapted in its application to metals having a high melting point, such as tool steel, because of the results achieved to be referred to in detail hereinafter and for the reason that the work from which the casting is formed is itself directly subjected to intense heat instead of heating the metal in a crucible or other apparatus for bringing it to molten condition.

Further and other objects and advantages of the invention will be apparent as the description thereof proceeds.

According to the preferred form of the invention, the metal as, for instance, steel or other material from which the casting is to be formed, is employed in the process in shaped or block form, as a rod or bar or a disc or roller and a portion thereof, such as an end or edge, is fused or brought to molten or liquid condition by the direct application of heat, such as for instance, by means of the well-known electric arc method and in which the metal material itself may form one of the electrodes. The end of the rod or bar, or if a disc or roller is employed, its periphery is then fused and forced quickly in molten condition, and while it remains an integral part of the rod or disc, into the die and pressure is then applied to the molten metal within the die, the pressure-applying means preferably being the un-molten or relatively cool portion of the metal work or material itself.

The several figures of the accompanying drawings show a practical embodiment of an apparatus by means of which the process of the invention may be practiced. In said drawings:

Fig. 1 is a top plan view of one form of such apparatus.

Fig. 2 is a side elevation thereof.

Fig. 3 is a vertical cross-section on the line 3—3 of Fig. 2.

Fig. 4 is a horizontal cross-section on the line 4—4 of Fig. 3.

Fig. 5 is a sectional view of a modified form of apparatus taken on the line 5—5 of Fig. 6, and

Fig. 6 is a vertical cross-section of the modification taken on the line 6—6 of Fig. 5.

Referring in detail to the drawings and, for the present, more particularly to Figs. 1 to 4 inclusive:

5 A walled chamber within which the process of the invention may be practiced is indicated at 10. Said chamber is provided with a base 11, a front wall 12 detachably secured to the chamber, as by screws 13, whereby access to the interior of the chamber may readily be had, and an inwardly extending annular flange, as shown, forming a bearing member for a work-holder as will be herein described. A rotatable work-holder is indicated at 15 and carries the work 16 from the lower end of which the casting is to be formed. In the preferred form of the invention the work comprises a rod or suitable fusible and preferably metallic material, such as steel. This steel 10 rod extends downwardly through the work-holder and into the chamber and it is slidably and adjustably held in said work-holder in any desirable manner, as by set-screw 17 passing through the work-holder and into clamping engagement 15 with the rod 16.

The upper end of the work-holder 15 is reduced in character as at 18 and extends through and is journalled within a cross-bar 19. The ends of said cross-bar are provided with guiding 25 pins 20 slidably received within slots 21 of angled vertical supporting arms 22, the angles of which are detachably secured to the upper portion or wall of the chamber by means of adjustable screws 23. Tension springs 24 are connected to 30 said screws and to the cross-bar 19 and constantly urge movement of the cross-bar 19 downwardly and accordingly movement of the work-holder 15 in the same direction with the guiding pins 20 engaging with the slots 21. A ball-race 35 25 may be provided and is interposed between the cross-bar 19 and work-holder 15 to decrease the effect of friction between the cross-bar 19 and work-holder 15 when the latter element is rotated. To permit connection between the cross-bar 40 19 and work-holder 15 while permitting rotation of the latter, I have provided a strap 25' fastened to the cross-bar and slidably engaging beneath an annular flange 25'' with which the work-holder is provided.

45 A rotatable sleeve is indicated at 26. Said sleeve is rotatably journalled within an inwardly extending flange or wall 27 which is preferably integral with the side walls of the chamber 10 and the sleeve is provided with an annular flange 50 28 acting as a stop to limit its upward vertical movement within said flange or wall 27. The sleeve 26 and work-holder 15 are splined together by means of a key 29 on the sleeve which enters a slot 30 in the work-holder. This connection 55 permits vertical movement downwardly of the

work-holder 15 within the sleeve but prevents relative rotation of one member with respect to the other.

The upper end of the sleeve 26 is provided with a toothed gear or pinion 31 detachably fastened thereto in any desirable manner whereby it is rotatable with said sleeve. The teeth of the pinion 31 mesh with the teeth of a slidable rack 32 guided in its movement by an angle-bar 33 which may be fastened to a wall of the chamber. One end of the rack is adapted to enter a suitable slot 34 in a wall of the chamber and the other end is provided with a shank 35 journalled in and extending through an opposite wall and terminating in an operating handle 36. Obviously, reciprocation of the rack 32 by the handle 36 will rotate the sleeve 26 and consequently the work-holder 15 which carries the rod 16 with it.

A slidable die-support comprising a plate, slideable on the base 11, is indicated at 37. Said support detachably carries a metallic die 38 thereon which contains the impression from which the casting is to be made. In its base the die is provided with suitable openings for frictionally receiving pins 39 whereby removal and substitutions of different dies may readily be made with facility after the detachable front wall 12 has first been removed. The die-support extends through an opening in a wall of the chamber with which it slidably interfits and the opposite wall is provided with a screw-threaded opening receiving an adjustable screw 40. Said screw acts as a stop to limit the movement to the left (Fig. 3) of the support 37 on the base 11 and by adjusting said screw, the die may be brought into exact vertical alignment with the work comprising the rod 16.

An actuating rod or bar is indicated at 41 and terminates in a handle 42. Said rod is pivoted at 42', as shown, to a bracket 43 fastened to a wall of the chamber and it is also connected by a pin and slot connection 44 to the die-support 37. A horizontally slidable rod comprising an electrode is indicated at 45. Said rod is slidably received by an insulating bushing 46 mounted in a wall of the chamber and it is pivotally connected to an end of actuating rod 41 by a pin and slot connection 47. Insulating material surrounds this last-named connection, as illustrated, to prevent short circuiting.

A bracket 48 is mounted on a wall of the housing and has an arm 49 pivoted thereto as at 49'. The lower end of said arm 49 engages a lug or projection 50 made of an insulating material and carried by the rod 45. The upper end of said arm 49 is connected by a pin and slot connection 51 to a locking arm 52 journalled in a wall of the housing and terminating at its inner end in a locking member 53 having an opening 54 of a size permitting it to normally loosely receive the work-holding member 15. One side of the opening 54 is bevelled as at 55 and is adapted to be received by an annular notch 56 in the member 15 to hold and detachably lock it in elevated position against the action of the springs 24. A compression spring 56' is interposed intermediate the arm 49 adjacent its upper end and a wall of the chamber and urges said arm to swing in a clockwise direction to retain the member 15 in raised and locked position.

A binding post is indicated at 57 and is provided with a shank entering a bore 58 extending through a wall of the chamber. A compression spring 59 is mounted in said bore intermediate the shank of the binding post and a termi-

nal 60 also mounted in the bore and having wiping electrical contact with the sleeve 26. A conductor 61 is fastened to the binding post 57 and is connected to a source of current supply (not shown) while another conductor 62 is also connected to said source of current supply and to the electrode 45.

The apparatus is shown in inoperative position with the metal die 38 shielded by a baffle plate 63 to prevent the introduction of dirt or other foreign matter into the die and which may be formed as an integral part of a wall of the chamber. I have also provided means for visual inspection of the end of the rod 16 in order to inspect its physical condition while being subjected to heat to bring it to molten condition. Said means comprises a tube 64 extending through the wall 12 and in horizontal alignment with the end of the rod 16. Mounted on the outer end of said tube exteriorly of the chamber is a head 65 carrying a transparent plate 66, preferably of glass. This arrangement prevents the entrance of air into the chamber which is desirable in some cases as I have often found it expedient to carry on operations within the chamber in a vacuum or partial vacuum to prevent scaling of the rod 16 or the casting to be formed therefrom and which also enhances the fusing operation by the electric arc method.

Assuming the parts are in the positions shown, the operation of the apparatus is as follows:

The rod 41 is thrown to the right on its pivot 42' (Fig. 3) in order to bring the inner end of the electrode 45 into contact with the lower end of the rod 16 to establish the completion of the electrical circuit through the end of the rod and the electrode. The rod 41 is then moved slightly to the left or in a clockwise direction to space the end of the rod 16 and the end of the electrode 45 whereby an electric heating arc between the members is established. Meanwhile fusing of the end of the rod 16 proceeds and while so proceeding the rack 33 is reciprocated backwardly and forwardly to thereby rotate the rod in an obvious manner and thereby secure a uniform fusion thereof at all places adjacent its lower end. When said end has reached the necessary molten state and before it has had an opportunity to solidify and just before it has fallen by gravity from the unmolten portion of the rod, as determined by visual inspection thereof in the manner previously described, the bar 41 is thrown completely to the left on its pivot in a clockwise direction and as indicated at the left in dotted lines in Fig. 3. This movement, obviously, carries the die 38 on its support 37 into vertical alignment with the end of the rod 16, retracts the electrode 45 and releases the locking edge 55 from its engagement with the notch 56 whereby the work-holder 15 is moved downwardly instantly within the sleeve 26 with great speed due to the action of the springs 24, and the molten metal on the end of the rod 16 is brought within the die 38 and is firmly compressed therein by the unfused or unmolten part of said rod 16 to form a "splash" casting which conforms in configuration to the inner configuration of the die 38.

Adhesion or sticking of the molten metal to the die is obviated because of the relatively large difference in temperature therebetween whereby a very sudden chilling and consequent contraction of the metal is effectively brought about immediately upon its contact with the die. After the casting is so formed, the work-holder 15 car-

trying the rod 16 with the formed casting on the end thereof is manually raised by means of the cross-bar 19 to its initial position and locked in that position by swinging the rod or bar to inoperative or vertical position shown in full lines in Fig. 3 to permit the action of the spring 56' to bring the holder 15 and locking member 53 into interlocked engagement. The formed casting may then be cut off from the end of rod 16 at any desired length. As the operating length of the rod 16 becomes shortened because of the successive fusions of its end and the formation of successive castings, its operating length may be lengthened whenever desired by loosening the set-screw 17 and forcing the rod downwardly within its holder. It will be found that castings produced by the process described herein do not require tempering as by re-heating and plunging in a cold liquid as they are sufficiently hardened or tempered by the quick cooling effect of the metallic die 38. This sudden chilling of the molten metal on the end of the rod 16, furthermore, prevents it from sticking to the die, as is obvious, and as has previously been explained.

In the modification illustrated in Figs. 5 and 6, the metal or other material from which the casting is formed is preferably in the form of a disc or roller indicated at 67 and is detachably mounted in any manner on a separable or two-part shaft 68 the ends of which are journaled in opposite walls of the chamber. The casting in this case becomes a part of the peripheral edge of said disc or roller. The shaft 68 is prevented from horizontal movement in one direction by a washer and set-screw indicated generally at 69 and the other end of the shaft is provided with a crank 70 for the purpose of rotating it.

An elongated die is indicated at 71 and is slidable or movable of its longitudinal axis. It extends within suitable slots 72 formed in the body of the chamber which guide the die in its movement. Said die is grooved as at 73 in its face or side adjacent the disc or roller 67, said groove being formed with or containing the object or inscription etc. which it is desired to reproduce by a casting. A bracket 74 is fastened to a wall of the chamber and a bar or rod 75 is pivoted thereto, as by pivot 76. The upper end of said bar is connected by a pin and slot connection 77 to a detent slide or rod 78 extending through an opening in a wall of the housing which slidably supports it. The inner end of said detent slide normally engages beneath the end of the die 71 to hold it in the inoperative or retracted position shown in the drawings.

A rod 79 is secured to the upper end of the die 71 or it may be integral therewith. Secured to the said rod 79 is a cross-arm 80 and tension springs 81 are fastened to said cross-arm adjacent its ends and to an upper wall of the chamber. The action of said springs 81 tend by their action to forcibly and expeditiously move the die 71 downwardly within the slots 72 as is obvious.

The bar or rod 75 terminates at its lower end in a handle 82 and said bar or rod is connected by a pin and slot connection 83 to an angle bar, the horizontal leg of which is indicated at 84 while its vertical leg is indicated at 85. The vertical leg 85 may be supported by a pin or bolt 86 extending loosely therethrough and into the body of the housing and a compression spring 87 encircles said pin or bolt and bears against said leg and housing and tends by its action to retain said leg a spaced distance from said housing.

A pin and slot connection 88 connects the upper end of the leg 85 to an electrode 89 slidably mounted in an insulated bushing 90 in a wall of the chamber, said pin and slot connection being surrounded by insulating material as in the previous case. A conductor 91 is connected to a source of current supply (not shown) and to the outer end of electrode 89 while conductor 92 is connected to the same source of current supply and to a wall of the chamber.

As in the previous case, the handle 82 is manipulated in the proper direction to bring the inner end of the electrode 89 into contact with the periphery of the disc or roller 67 to establish an electrical circuit. It is then again manipulated slightly to space the roller from the end of the electrode whereby a heating electric arc is established to fuse the peripheral edge of the disc or roller. When the fusing of such edge has been completed and just before the fused metal falls of its own weight by gravity, the handle is swung in such manner as to release the detent 78 from engagement with the die or mold 71 which travels downwardly under the influence of springs 81 and the fused metal on the peripheral edges of the disc or roller 67 enters the groove 73 in the die to form the desired casting. The unfused and comparatively cool portion of the disc provides sufficient pressure and resistance for the formation of the casting on the edge of the disc. Said disc, with the finished casting thereon, is then removed and a new one substituted for repetition of the same operation. As in the previous case, the cool die prevents the fused metal on the edge of the disc from sticking thereto.

I have shown in this modification a device for feeding a powdered carbonized material to the fusing metal for hardening the metal and casting which obviously could be employed in the preferred form of apparatus, if so desired, and in fact it is preferred to so employ it. A hopper 93 for holding the powdered carbonized material 94 is fastened to a wall of the chamber by brackets 95. This hopper interconnects with a feed tube 96 directed toward the peripheral edge of the disc or roller 67. The passageway between the hopper and tube may be open or closed by a handled spindle or plunger 97. Just as about the edge of the disc or roller 67 has reached fused condition the carbonized material is permitted to fall thereon by opening the connection between the hopper and feed tube 96, while the disc or roller 67 is continuously rotated by the crank 70.

This application is a division of my prior application for patent for Apparatus for producing castings, filed April 18, 1940, Ser. No. 330,287, allowed June 3, 1942.

The invention claimed is:

1. The process of producing a metallic casting consisting in providing a solid mass of metal having substantially the same physical properties therethroughout and provided with a free and unsupported portion from which the casting is to be made, heating said unsupported portion of said metal to reduce the same to a molten state, bringing such molten portion of the metal into contact with a cooling die while it remains integral with the unmolten portion of the metal to suddenly chill it and simultaneously compressing the molten portion of the metal against the die by pressure applied by the unmolten portion of the metal to form a "splash" casting integral with said unmolten portion conforming in con-

figuration with the inner configuration of said cooling die.

2. The process of producing a metallic casting consisting in providing a mass of metal from which the casting is to be made and having substantially the same physical properties therethroughout, rotating said mass of metal, subjecting an edge portion of said metal to heat to reduce the same to a molten state, bringing the molten portion of the metal while integral with the unmolten portion thereof into contact with a cooling die to suddenly chill it and simultaneously compressing the molten portion of the metal against the die by pressure applied by the unmolten portion of the metal to form a "splash" casting integral with said unmolten portion conforming in configuration with the inner configuration of said cooling die.

3. The process of producing a casting consisting in providing a rod of metal from which the casting is to be made and having substantially the same physical properties therethroughout, subjecting an end of said metal rod to heat and reducing the same to molten condition, bringing the molten end of the rod downwardly into contact with a cooling die by mechanical means assisted by gravity while said molten end is integral with said rod simultaneously applying pressure to the unmolten body of the rod to compress the molten end against the die to form a splash casting conforming in configuration to the configuration of said cooling die and removing the casting so formed to retain the untreated portion of said rod for the production of successive castings by a like process.

4. The process of producing a casting consisting in providing a metallic rod having substantially the same physical properties therethroughout, subjecting an end of said rod to heat to fuse the same, forcing the fused end of said rod downwardly into contact with a cooling die while it remains integral with said rod, applying pressure to the unfused body of the rod to force the fused end against said die to effect a sudden chilling of said fused end and form a splash casting on the end of the rod and then removing the casting so formed from the body of the rod to retain the untreated portion of said rod for the production of successive castings by a like process.

5. The process of producing a casting consisting in providing a metallic rod having substantially the same physical properties therethroughout, subjecting an end of said rod to fusing temperature by the electric arc process while rotating said rod, discontinuing the heating and rotation of the rod when the end of the rod is reduced to a molten state and then subjecting the molten portion of the rod to the action of a forming and cooling die for suddenly chilling it and shaping it into the desired form by pressure

applied by the unfused portion of said rod while it remains integral with the body of the rod.

6. The process of producing a casting consisting in providing a mass of metal having substantially the same physical properties therethroughout, subjecting an edge of said mass to fusing temperature while simultaneously applying powdered carbonized material to said fusing edge, forcing the fused metal so treated to enter a cooling die and subjecting the fused metal within the die to pressure applied by the unfused portion of said mass.

7. The process of producing a casting consisting in providing a solid mass of metal having substantially the same physical properties therethroughout, subjecting a portion of said mass to fusing temperature within a partial vacuum and reducing such portion of the mass to a molten state, disposing the molten portion of the mass in a cooling die and simultaneously applying pressure to the unmolten portion of said mass to compress the molten portion within the die to form a "splash" casting integral with said unmolten portion.

8. The process of producing a casting consisting in providing a disc of metal, subjecting the periphery of said disc to fusing temperature while rotating said disc and moving a die into contact with the fused peripheral edge of said disc.

9. The process of producing a casting consisting in providing a mass of metal having substantially the same physical properties therethroughout and from a portion of which the casting is to be produced, rotating said mass, subjecting an edge portion thereof to heat, discontinuing said rotation and heating when said edge portion has been reduced to a molten condition, forcing said molten portion while it remains integral with the unmolten portion into contact with a cooling die and compressing said molten portion within the die by pressure applied thereagainst by said unmolten portion to suddenly chill said molten portion and to form a "splash" casting integral with said unmolten portion.

10. The process of producing a casting consisting in providing a metallic rod having substantially the same physical characteristics therethroughout and from an end of which the casting is to be produced, rotating said rod, subjecting an end of said rod to heat within a partial vacuum to reduce said end to molten condition while retaining the body of the rod in unmolten condition, discontinuing said rotation and heating and moving the rod to force the molten end thereof into contact with a cooling die to compress said molten end within said die by pressure applied thereagainst by said unmolten body to suddenly chill said unmolten portion and thereby form a "splash" casting on the end of said rod.

JOSEPH E. JOHNSON.